

Oct. 30, 1945.

R. A. PICKENS

2,387,856

RECOVERY OF ILMENITE BY TWO STAGE FLOTATION PROCESSES

Filed May 26, 1942

2 Sheets-Sheet 1



Oct. 30, 1945.

R. A. PICKENS

2,387,856

RECOVERY OF ILMENITE BY TWO STAGE FLOTATION PROCESSES

Filed May 26, 1942

2 Sheets-Sheet 2



## UNITED STATES PATENT OFFICE

2,387,856

## RECOVERY OF ILMENITE BY A TWO-STAGE FLOTATION PROCESS

Roy Alderson Pickens, Stamford, Conn., assignor to American Cyanamid Company, New York, N. Y., a corporation of Maine

Application May 26, 1942, Serial No. 444,500.

3 Claims. (Cl. 209—166)

This invention relates to froth flotation of ores particularly to the beneficiation of ilmenite ores by a two stage flotation process.

In commercial practice the use of titanium has become more and more important and accordingly the demand for a high grade ore from which it may be recovered has steadily increased. To carry out a satisfactory recovery it is necessary to have an ore or a concentrate containing at least 50% of a titanium bearing mineral such as ilmenite, rutile and the like. While there are many deposits of titanium ores in the United States, the grade in most cases is not sufficiently high to make the recovery of titanium economically feasible. As a consequence, in the past a large proportion of the titanium used was obtained from imported ores.

In order to make use of the domestic ores, it has been proposed to beneficiate them by froth flotation to produce a concentrate of satisfactory grade for further processing. Attempts have been made to float the ilmenite away from the impurities by the use of anionic reagents such as oleic acid, sodium oleate, talloel, talloel soap, fish oil, fatty acids, anionic-type wetting agents and the like. It was found, however, that successful concentration to the desired grade required an initial ore of fairly high grade and extremely careful control of both the amount of reagent used and the flotation conditions. If any of these factors were allowed to vary from rather exacting requirements an unsatisfactory separation was obtained. As a result, the anionic flotation was neither particularly useful nor desirable on a commercial scale for the beneficiation of many naturally-occurring ores.

Attempts have also been made to float the impurities such as talc, chlorite and other silicate-bearing materials which usually comprise the undesirable portions of low grade native ores away from the ilmenite by the use of a cationic reagent. When using a cationic-type of reagent alone it was found that with fairly high grade ore as the initial starting material a satisfactory concentration could be obtained, although often at the expense of good recovery. However, the concentrate so produced was in a wholly unsatisfactory physical condition since it could be neither readily filtered nor dried without resorting to equipment and a degree of care in their use which would render the process commercially undesirable.

Most of the lower grade ilmenite ores which require beneficiation in order to produce a marketable product, fall within one of three classes.

The first of these comprises those ores of a sufficiently high initial grade so that a marketable grade can be obtained in a single step flotation either by floating the silicate-bearing materials away from the ilmenite ores or alternatively floating the ilmenite away from the gangue with an anionic reagent. The present invention is not concerned with ores of this high an initial grade.

The second of these classes comprises those ores which permit a part of the finished product to be produced as tailings from a rougher silicate flotation and the remainder must be obtained by a retreatment of the rougher silicate concentrate. Ores of this type will be referred to in the succeeding portions of the present specification as easily-beneficiated ores.

The third of these classes comprises those ores which in order to produce a marketable grade require further treatment of both the rougher silicate tail and the rougher silicate concentrate. Ores of this type will be referred to throughout the specification as difficultly beneficiated ores.

According to the present invention it is possible to produce concentrates which are of satisfactorily high grade with a good recovery and also have the concentrate in such physical condition that it can be readily filtered and dried. This is accomplished in general by the use of a two-stage flotation process in which a portion of the silicates and silica are removed by flotation with a cationic type of reagent after which the ilmenite is concentrated by flotation with an anionic type of reagent.

The invention is most readily set forth in connection with the accompanying drawings in which:

Figure 1 is a flow sheet showing the procedure used with an ore which is relatively free from difficultly-separable, undesirable portions; and

Figure 2 is a flow sheet of the procedure used with an ore containing a fairly large amount of impurities which can be removed only with great difficulty.

In connection with both Figures 1 and 2, it may be noted that the present process is considered as starting with a flotation feed which has been previously ground. The ore, as mined, is in varied states of aggregation from fines to large lumps. Since the material must be ground for flotation, the process for the purpose of this application is considered as starting with all the ore ground or crushed to pass a screen of designated fineness, for example 10 mesh.

Also in both figures it will be noted that the first flotation stage is a silicate rougher flota-

tion using a cationic reagent. Since the cationic reagents are extremely sensitive to the presence of slimes, even small amounts of the latter seriously impairing the efficiency of the reagent, it is necessary to remove as large a proportion of the slimes as practicable before this first flotation step. If desired, a preliminary desliming may be carried out on the ore after it has been crushed and before fine grinding although it is unnecessary to do so in all cases.

In preparing the ore for desliming, a procedure which produces good results is to wet grind the previously crushed ore with a sufficient amount of an alkaline material such as caustic soda or soda ash to maintain the liquid in the grinding apparatus at a basic pH. The grinding may be carried out in any desired form of apparatus. Good results may be obtained using almost any commercial form of rod or ball mill. In some instances I have found that it is desirable to grind the material until about 1% is retained on a 65 mesh screen and 48-50% will pass a 200 mesh screen, although the process need not be limited to this degree of grinding. Excessive grinding should be avoided since it tends to increase the amount of titanium mineral removed with the slimes and thereby lost.

The ground ore is then subjected to a desliming procedure. Again the type of apparatus used is immaterial and the operation may be carried out for example either by hydraulic classification or by means of a series of wet screens. Hydraulic classification is probably the quickest and easiest means and therefore, is perhaps preferable. The desliming, as was set forth above, should be carried out to the greatest extent that is feasible under the existing conditions since the more complete the desliming the more efficient will be the action of the cationic reagent used in the first flotation step.

After desliming, as will be noted in both Figures 1 and 2, the sands are passed to a flotation machine or a battery of flotation machines which may be of any desired type such as the well known Fagergren flotation machine. In some cases it has been found advisable in connection with the silicate rougher flotation to condition the pulp for a few seconds before adding the reagents, in this case a frother and a promoter of the cationic type.

An advantage of the present invention is that neither stage is limited to any particular reagents, any desired frothers and any desired cationic or anionic type promoters being satisfactory in the first and second stages respectively. For example, well-known frothers such as pine oil, cresylic acids and a mixture of higher alcohols known to the trade as "B-23," comprising principally C<sub>7</sub> and C<sub>8</sub>, have been found to produce excellent results. In the first stage, any desired cationic type of flotation reagent such for example as the quaternary ammonium reagents, the higher aliphatic amines or their salts and the reaction products of polyamines with higher aliphatic carboxylic acids may be used. All produce satisfactory results when used according to the process of the present invention.

With different ores, different cationic reagents may show slightly superior results. However, it is an advantage of the present invention that this factor need not be considered. If only the cationic float were to be used, great care would necessarily be employed in selecting the optimum amounts of the best agent. But since this is not true of the present process in which the cationic

flotation is in effect a preliminary treatment, this degree of care is not necessary. Any available reagent may be used so that the cheapest is the most preferable. At the same time, the minimum amount of reagent may be used. Since these reagents are fairly expensive, this feature of the invention is of considerable importance.

Referring to Figure 1, delineating the procedure suitable for easily concentrated ores, the silicate concentrate from the silicate rougher flotation is subjected to a cleaning flotation and if so desired to one or more recleaner silicate flotation operations. Since the cleaned silicate concentrates are usually relatively free from ilmenite, they may usually be discarded without appreciable loss. However, it is possible to recover at least a portion of any ilmenite retained in the recleaned silicate concentrate by regrinding and reclassifying it, discarding the overflow and returning the underflow to the silicate rougher flotation stage.

The tailings from the silicate rougher flotation with easily beneficiated ores of this type are usually of sufficiently high grade to constitute a finished product. With some few ores the tailings from the silicate cleaner flotation may also be added directly to the silicate rougher tail without causing the latter to fall below the desired grade. However, as previously pointed out, the present invention is not concerned with ores of that high an initial grade since thereby the whole ilmenite flotation is by-passed and the process of the present invention is not required in the beneficiation of such ores.

With ores of the type with which the present invention is concerned, however, the tailings from the several silicate cleaner floatations are combined and subjected to an ilmenite rougher flotation with a flotation reagent of the anionic type. Again the particular reagent used is not critical. Good results may be obtained using such well-known reagents for example, as oleic acid, cocoanut oil fatty acid, talloel, saponified fatty acids and saponified talloel, although the invention is not meant to be limited to these particular reagents since others of a similar nature may be used. The tailings from the ilmenite rougher flotation itself may be discarded or if the ilmenite content is high enough to warrant further treatment, this material may be retreated by any of the usual methods of concentration including flotation or gravity concentration, either directly or after regrinding.

Naturally, if the concentrate from the ilmenite rougher flotation is of sufficiently high grade no cleaning steps are required. Ordinarily however the concentrate is passed to one or more cleaning stages the final concentrate from which is the finished product and the tailings from which may be discarded or may be combined and retreated by methods similar to that previously described for the treatment of the rougher tailings.

By this two-stage flotation procedure ores which otherwise could not be beneficiated may be successfully used and ores of greatly varying grades may be fed to this process and still produce a product of satisfactory grade with a good recovery.

A further advantage with the two-stage flotation procedure lies in the fact that although in the case of easily treated ores only the initial silicate flotation step may be necessary in order to obtain the desired grade of ilmenite concentrate, such tailing from the silicate rougher flotation may not be in particularly good physical

state for subsequent dewatering and drying. In such cases it may be advisable to refloat this portion along with the tailings from the silicate cleaner and recleaner stages in order to take advantage of the improvement in physical state made by the anionic flotation.

This procedure will be illustrated by the following example which is meant to be merely illustrative and in no way limit the present invention. All parts are by weight.

#### EXAMPLE 1

1200 parts of a North Carolina ilmenite ore were crushed to pass a 10 mesh screen, diluted to about 67% solids, ground in a small rod mill for 13 minutes with 1.25 lbs./ton of caustic soda and then deslimed by decantation. The deslimed sands were diluted to 33% solids, conditioned for about 10 seconds with 0.125 lb./ton of pine oil and 0.125 lb./ton of "Lorol" amine hydrochloride, a commercial product comprising principally lauryl amine hydrochloride and well-known to the trade as D. P.-243, and floated for 2 minutes in a Fagergren flotation machine. The concentrate was given a cleaning and a recleaning float of 2 minutes each with 0.02 lb./ton of "Lorol" amine hydrochloride. The rougher silicate tail was a finished product and was not further treated. The cleaner and recleaner silicate tails were combined, diluted to 30% solids, conditioned for about 30 seconds with 0.12 lb./ton of oleic acid and floated for 4 minutes with 0.07 lb./ton of additional oleic acid. The ilmenite rougher concentrate was given a cleaning and recleaning float of 2 minutes each, without reagents, and an additional recleaner float with 0.03 lb./ton of oleic acid. The results are shown in Table I.

Table I

|                                                                    | Percent weight | Assay percent $TiO_2$ | Percent dist. $TiO_2$ |
|--------------------------------------------------------------------|----------------|-----------------------|-----------------------|
| Feed                                                               | 100.00         | 42.20                 | 100.00                |
| Slime (waste)                                                      | 24.43          | 22.43                 | 12.98*                |
| Sand (floatation feed)                                             | 75.57          | 48.59                 | 87.02                 |
| Silicate rougher conc.                                             | 52.39          | 45.87                 | 56.94                 |
| Silicate rougher tail                                              | 23.18          | 54.76                 | 30.08                 |
| Silicate recleaner conc. (waste)                                   | 7.38           | 19.75                 | 3.46                  |
| Combined silicate cleaner tails (ilmenite rougher feed)            | 45.01          | 50.15                 | 53.48                 |
| Ilmenite rougher conc.                                             | 39.81          | 52.80                 | 49.80                 |
| Ilmenite rougher tail                                              | 5.20           | 29.87                 | 3.68                  |
| Ilmenite recleaner conc.                                           | 33.35          | 53.97                 | 42.65                 |
| Ilmenite recleaner tail (middlings)                                | 6.46           | 46.74                 | 7.15                  |
| <i>Product combinations</i>                                        |                |                       |                       |
| Silicate rougher tail+ilmenite recleaner conc.                     | 56.53          | 54.29                 | 72.73                 |
| Silicate rougher tail+ilmenite recleaner conc. +ilmenite middlings | 62.99          | 53.52                 | 79.88                 |

Figure 2 is a flow sheet which represents the procedure with an ore which contains a large proportion of difficultly removable impurities such as weathered chlorite and certain forms of iron bearing minerals. The ore is prepared in the same way, by grinding and desliming and the same flotation reagents are used as in the procedure outlined in Figure 1. With these difficultly beneficiated ores, the principal changes in procedure lie in the manner in which various concentrates are combined to make up the product and in the manner in which various tailings may be reworked. The silicate rougher concentrate is passed to a cleaner silicate flotation and the concentrate therefrom subjected to one or more silicate recleaner stages. The tailings from

the rougher silicate float instead of being a finished product are combined with the tailings from the recleaner stages and subjected to a rougher ilmenite flotation with an anionic type of reagent. The tailings from the rougher ilmenite float are usually fairly high in titanium content and consequently may advantageously be retreated, although if the titanium content is low they may be discarded. The ilmenite rougher concentrate may be of sufficiently high grade to be finished product, although ores in which this is possible are seldom encountered. It is usually advantageous to subject the ilmenite rougher concentrate to one or more cleaning stages, the concentrate from the final stage of which forms the product. The combined tailings from the cleaner stages should ordinarily be recycled to the rougher ilmenite float to recover part of their titanium content. However, if the tailings comprise a large amount of fine titanium ore physically bound to impurities, it may be well to regrind these tailings prior to further treatment.

This modification of the procedure will be illustrated by the following examples which are also meant to be merely illustrative and not by way of limitation. All parts are by weight.

#### EXAMPLE 2

1200 parts of an ilmenite ore composite were diluted with 600 parts of water containing 1.5 lbs./ton of caustic soda, ground in a rod mill for about 13 minutes and deslimed by three successive decantations. The deslimed sands were given a rougher silicate float at about 35% solids by conditioning for 5 seconds and then floating for 2 minutes with 0.06 lb./ton of pine oil and 0.2 lb./ton of the reaction product of thiourea and  $\beta$ -chlorethylololeate, a cationic type reagent. The silicate rougher concentrate was given a cleaning and recleaning float of 3 minutes each and the recleaned silicate concentrate discarded. The silicate rougher tail was combined with the tailings from the cleaner and recleaner floats, diluted to about 30% solids, conditioned for 45 seconds and floated for 2½ minutes with 0.12 lb./ton oleic acid. The ilmenite concentrate was cleaned once. The metallurgical results are shown in Table II.

Table II

|                                                                             | Per cent wt. | Assay per cent $TiO_2$ | Per cent dist. $TiO_2$ |
|-----------------------------------------------------------------------------|--------------|------------------------|------------------------|
| Feed                                                                        | 100.00       | 43.47                  | 100.00                 |
| Slime (waste)                                                               | 20.36        | 21.42                  | 20.04                  |
| Sand (floatation feed)                                                      | 79.64        | 49.11                  | 89.96                  |
| Silicate reclean. conc.                                                     | 2.67         | 28.25                  | 1.73                   |
| Silicate rough. tail+combined silicate clean. tails (ilmenite rougher feed) | 76.97        | 49.83                  | 88.23                  |
| Ilmenite rough. tail                                                        | 13.39        | 39.67                  | 12.03                  |
| Ilmenite clean. tail                                                        | 7.23         | 46.24                  | 7.69                   |
| <i>Product</i>                                                              |              |                        |                        |
| Ilmenite clean. conc.                                                       | 56.35        | 52.85                  | 68.51                  |

#### EXAMPLE 3

The procedure of Example 2 was repeated using 0.06 lb./ton of B-23 and 0.08 lb./ton of an aliphatic amine hydrochloride, principally octadecyl amine and known to the trade as "Armour" amine hydrochloride, in the cationic float and 0.7 lb./ton of oleic acid in the anionic float. The cleaner and recleaner silicate tails, however, were

not combined with the rougher silicate tail from the anionic float but were discarded since they contained negligible quantities of titanium. The results are shown in Table III.

Table III

|                                             | Per cent wt. | Assay per cent $\text{TiO}_2$ | Per cent dist. $\text{TiO}_2$ |
|---------------------------------------------|--------------|-------------------------------|-------------------------------|
| Feed                                        | 100.00       | 43.39                         | 100.00                        |
| Slime (white)                               | 20.12        | 21.64                         | 10.03                         |
| Sand (flotation feed)                       | 79.88        | 48.87                         | 89.97                         |
| Silicate rough. conc.                       | 5.13         | 14.44                         | 1.71                          |
| Silicate rough. tail (ilmenite rough. feed) | 74.75        | 51.23                         | 88.26                         |
| Ilmenite rough. tail                        | 20.30        | 44.42                         | 20.78                         |
| Ilmenite clean. tail                        | 5.92         | 48.29                         | 6.59                          |
| <i>Product</i>                              |              |                               |                               |
| Ilmenite clean. conc.                       | 48.53        | 54.44                         | 60.89                         |

EXAMPLE 4

The procedure of Example 3 was repeated using 0.06 lb./ton of pine oil and 0.10 lb./ton of "Lorol" amine hydrochloride in the cationic float and 1.0 lb./ton of saponified talloel in the anionic float. The results are shown in Table IV.

Table IV

|                                               | Per cent wt. | Assay per cent $\text{TiO}_2$ | Per cent dist. $\text{TiO}_2$ |
|-----------------------------------------------|--------------|-------------------------------|-------------------------------|
| Feed                                          | 100.00       | 41.79                         | 100.00                        |
| Slime (waste)                                 | 20.38        | 20.42                         | 9.96                          |
| Sand (flotation feed)                         | 79.62        | 47.26                         | 90.04                         |
| Silicate clean. conc.                         | 14.10        | 29.61                         | 9.99                          |
| Silicate comb. tail (ilmenite flotation feed) | 65.52        | 51.06                         | 80.05                         |
| Ilmenite rough. tail                          | 5.81         | 34.17                         | 4.75                          |
| Ilmenite clean. tail                          | 3.81         | 50.57                         | 4.61                          |
| <i>Product</i>                                |              |                               |                               |
| Ilmenite clean. conc.                         | 55.90        | 52.85                         | 70.69                         |

EXAMPLE 5

The procedure of Example 3 was repeated using 0.24 lb./ton of the acetate of the reaction product of mixed polyethylene polyamines and coconut oil fatty acid in the silicate rougher float and 1.0 lb./ton of Black Liquor Soap in the ilmenite rougher float. The results are shown in Table V.

Table V

|                                               | Percent wt. | Assay percent $\text{TiO}_2$ | Percent dist. $\text{TiO}_2$ |
|-----------------------------------------------|-------------|------------------------------|------------------------------|
| Feed                                          | 100.00      | 42.34                        | 100.00                       |
| Slime (waste)                                 | 20.32       | 20.42                        | 9.83                         |
| Sand (flotation feed)                         | 79.68       | 47.75                        | 90.17                        |
| Silicate clean. conc. (waste)                 | 4.27        | 27.34                        | 2.76                         |
| Silicate comb. tail (ilmenite flotation feed) | 75.35       | 49.12                        | 87.41                        |
| Ilmenite rough. tail                          | 27.57       | 46.93                        | 30.56                        |
| Ilmenite clean. tail                          | 5.67        | 45.56                        | 6.10                         |
| <i>Product</i>                                |             |                              |                              |
| Ilmenite clean. conc.                         | 42.11       | 51.05                        | 50.75                        |

EXAMPLE 6

The procedure of Example 3 was repeated using 0.35 lb./ton of trimethylcetyl ammonium bromide in the cationic float and 0.3 lb./ton of oleic acid in the anionic float. The results are shown in Table VI.

Table VI

|                                               | Percent wt. | Assay percent $\text{TiO}_2$ | Percent dist. $\text{TiO}_2$ |
|-----------------------------------------------|-------------|------------------------------|------------------------------|
| 10                                            |             |                              |                              |
| Feed                                          | 100.00      | 43.13                        | 100.00                       |
| Slime                                         | 20.38       | 20.42                        | 9.65                         |
| Sand (flotation feed)                         | 79.62       | 48.94                        | 2.16                         |
| 15                                            |             |                              |                              |
| Silicate clean. conc. (waste)                 | 3.02        | 30.75                        |                              |
| Silicate comb. tail (ilmenite flotation feed) | 76.60       | 49.66                        | 88.20                        |
| Ilmenite rough. tail                          | 13.16       | 41.00                        | 12.51                        |
| Ilmenite clean. tail                          | 8.58        | 46.93                        | 9.34                         |
| <i>Product</i>                                |             |                              |                              |
| 20                                            |             |                              |                              |
| Ilmenite clean. conc.                         | 54.86       | 52.16                        | 66.25                        |

I claim:

1. A process of beneficiating low grade ilmenite ores to produce a beneficiated ore adapted to ready filtration and drying and assaying at least 50%  $\text{TiO}_2$  which comprises subjecting the ore to a rougher silicate flotation in the presence of an amount of a cationic-type collector effective to concentrate a major portion of the silicates but insufficient to effect a maximum separation, whereby a concentrate rich in silicates and a tail rich in ilmenite are obtained, subjecting the rougher silicate concentrate to at least one silica cleaner flotation and subjecting at least a part of the silicate cleaner tailing to a rougher ilmenite flotation in the presence of an anionic collector selected from the group consisting of the higher fatty acids, talloel and soaps thereof.

2. A method according to claim 1 in which the silicate rougher flotation tailing and the silica cleaner tailing are combined as feed to the ilmenite rougher flotation.

3. A process of beneficiating low grade ilmenite ores to produce a beneficiated ore adapted to ready filtration and drying and assaying at least 50%  $\text{TiO}_2$  which comprises grinding the ilmenite ore in the presence of an alkaline material to a size suitable for froth flotation feed, desliming the ground ore in the presence of water, subjecting the deslimed ore to a rougher silicate flotation in the presence of an amount of a cationic-type collector effective to concentrate a major portion of the silicates but insufficient to effect a maximum separation, whereby a concentrate rich in silicates and a tail rich in ilmenite are obtained, subjecting the rougher silicate concentrate to at least one silica cleaner flotation and subjecting at least a part of the silicate cleaner tailing to a rougher ilmenite flotation in the presence of an anionic collector selected from the group consisting of the higher fatty acids, talloel and soaps thereof.

5. A process of beneficiating low grade ilmenite ores to produce a beneficiated ore adapted to ready filtration and drying and assaying at least 50%  $\text{TiO}_2$  which comprises subjecting the ground ore in the presence of water, subjecting the deslimed ore to a rougher silicate flotation in the presence of an amount of a cationic-type collector effective to concentrate a major portion of the silicates but insufficient to effect a maximum separation, whereby a concentrate rich in silicates and a tail rich in ilmenite are obtained, subjecting the rougher silicate concentrate to at least one silica cleaner flotation and subjecting at least a part of the silicate cleaner tailing to a rougher ilmenite flotation in the presence of an anionic collector selected from the group consisting of the higher fatty acids, talloel and soaps thereof.

ROY ALDERSON PICKENS.